

## UNITED STATES PATENT OFFICE.

WALTHER SCHMIDT, OF BITTERFIELD, GERMANY, ASSIGNEE TO I. G. FARBEINDUSTRIE AKTIENGESELLSCHAFT, OF FRANKFORT-ON-THE-MAIN, GERMANY.

## METHOD OF PRODUCING MAGNESIUM-SILICON ALLOY.

No Drawing. Application filed November 15, 1923, Serial No. 674,956, and in Germany November 17, 1923.

My invention refers to alloys of magnesium and silicon and its particular object is to produce alloys of this kind by the use of ferrosilicon, the resulting alloy being technically free from iron.

Up till now, alloys of magnesium and silicon were obtained either by mixing magnesium powder with quartz meal, causing these two bodies to react with one another, 10 or by introducing quartz meal into fluid magnesium and heating the melt to the temperature of reaction. This reaction mainly proceeds according to the formula:



15 The magnesium silicide thus obtained is dissolved in the metal in excess.

This method embodies several drawbacks, one of which is the considerable loss in magnesium, half of which is converted into magnesia. Moreover, unreduced particles of 20 silica remain in the alloy, such particles exerting an obnoxious influence, when the alloy is subjected to mechanical treatment.

25 It is further possible to produce alloys of the kind aforesaid by directly adding silicon to molten magnesium. However, this manner of proceeding also involves great disadvantages, insomuch as it requires heating to high temperatures, whereby a great 30 percentage of magnesium is oxidized or distilled over. The high price of elementary silicon also acts towards rendering this method uncommercial.

35 It is well known to those skilled in the art that molten ferro-silicon is capable of taking up magnesium and forming alloys of magnesium, iron and silicon, the constitution of which has not as yet been ascertained.

40 I have now discovered that the addition of greater quantities of magnesium to alloys of the kind mentioned has the unexpected effect of displacing the iron in the alloys to 45 such an extent that a separation of the alloy into a magnesium silicon alloy on the one hand and iron on the other hand takes place. As a rule, this will occur the easier, the higher, ranging from about 20 to 80 per 50 cent silicon, the percentage of silicon in the ferrosilicon employed and the greater the percentage of magnesium in the alloy of magnesium and silicon. At the end of the reaction, the alloy only contains so little iron (for instance 0.04 percent) that it can

practically be regarded as being entirely free from iron. In order to prevent the iron, which separates out, from being mechanically included, I prefer removing it during the formation of the alloy by acting upon it 60 with a slag-forming salt, for instance magnesium chloride.

In practising my invention, I may for instance proceed as follows:

I add to the molten magnesium the pre-determined quantity of ferro-silicon, this ferro-silicon containing from 35 to 70 per cent silicon; preferably the molten alloy is slightly overheated.

To this latter end, I add to a certain quantity of molten magnesium such quantities of preferably finely ground and powdered ferro-silicon as are required by the desired percentage of silicon in the alloy to be formed, the reaction being based solely on 75 the amount of silicon contained in the ferro-silicon. For instance a ferro-silicon of 33.8% Si will react according to the formula



80

It is advisable to use a certain surplus of ferro-silicon so as to meet the regular loss in the course of the process which is but small.

In order, for instance, to produce a magnesium-silicon alloy containing about 10% silicon, I proceed as follows:

10 kilos magnesium are heated to 800° C., which is about 150° above the melting point of pure magnesium. I then add about 2.5 kilos of finely powdered ferro-silicon containing 50% silicon, the powder being thoroughly mixed with the melt. The reaction which sets in immediately results in the formation of about 4 kilos of silicide of magnesium ( $\text{Mg}_2\text{Si}$ ), which remains dissolved in 95 the magnesium in excess, the alloy containing about 10% of silicon, as desired, while the iron remains undissolved and may be removed in any suitable manner, preferably by adding a slag-forming salt, such as magnesium-chloride, as mentioned above.

The higher the desired percentage of silicon in the terminal product, the higher the melt should be heated during the formation of  $\text{Mg}_2\text{Si}$ . I have found that the most favorable temperature of reaction rises steadily from 650° to 900° C. for a desired percentage of from 0 to 15% of silicon, a temperature of 900° C. corresponding to 15% silicon in the terminal product. However, in carry- 110

ing out my invention, I do not wish to be bound to these temperatures.

By thus proceeding, I obtain in a simple manner alloys of magnesium and silicon containing up to 15 percent silicon.

I wish it to be understood that I do not desire to be limited to the exact proportions and sequences of operations described, for obvious modifications will occur to a person skilled in the art.

I claim:—

1. The method of producing alloys of magnesium and silicon containing up to 15 percent silicon and being technically free from iron comprising causing a compound containing iron and at least 20 per cent silicon to react with an excess of molten metallic magnesium.

2. The method of producing alloys of magnesium and silicon containing up to 15 percent silicon and being technically free from iron, comprising causing a compound containing iron and at least 20 per cent silicon to react with an excess of molten metallic magnesium and removing the iron displaced.

3. The method of producing alloys of magnesium and silicon containing up to 15 percent silicon and being technically free from iron comprising causing ferro-silicon to react with an excess of molten metallic magnesium.

4. The method of producing alloys of magnesium and silicon containing up to 15 percent silicon and being technically free from iron comprising causing ferro-silicon containing at least 35 percent silicon to react with an excess of molten metallic magnesium.

40 5. The method of producing alloys of magnesium and silicon containing up to 15 percent silicon and being technically free

from iron, comprising introducing ferro-silicon into an excess of molten magnesium and slightly overheating the melt.

45

6. The method of producing alloys of magnesium and silicon containing up to 15 percent silicon and being technically free from iron, comprising introducing ferro-silicon powder into an excess of molten magnesium and slightly overheating the melt, the quantity of ferro-silicon employed being slightly in excess of the theoretical quantity.

50

7. The method of producing alloys of magnesium and silicon containing up to 15 percent silicon and being technically free from iron, comprising adding to 10 parts by weight of molten magnesium 2.5 parts of finely powdered ferro-silicon containing about 50 percent silicon, thoroughly mixing 60 the powder with the molten metal and removing the iron.

55

8. The method of producing alloys of magnesium and silicon containing up to 15 percent silicon and being technically free 65 from iron, comprising heating 10 parts by weight of magnesium to about 800° C., adding 2.5 parts of finely powdered ferro-silicon containing about 50 percent silicon, thoroughly mixing the powder with the molten 70 metal and adding a slag-forming salt to remove the iron.

70

9. The method of producing alloys of magnesium and silicon containing up to 15 percent silicon and being technically free 75 from iron, comprising heating 10 parts by weight of magnesium to about 800° C., adding 2.5 parts of finely powdered ferro-silicon containing about 50 percent silicon, thoroughly mixing the powder with the molten metal and adding magnesium chloride to remove the iron.

In testimony whereof I affix my signature.  
WALTHER SCHMIDT.